

May 9, 1939.

S. C. HIGHT

2,157,701

## PIEZOELECTRIC APPARATUS

Filed May 19, 1936

2 Sheets-Sheet 1

FIG. I



FIG. 2



FIG. 3



FIG. 4

FIG. 5



FIG. 6



INVENTOR  
S.C. HIGHT

W. J. O'Neill  
ATTORNEY

May 9, 1939.

S. C. HIGHT

2,157,701

PIEZOELECTRIC APPARATUS

Filed May 19, 1936

2 Sheets-Sheet 2



FIG. 10



FIG. 12

INVENTOR  
S.C. HIGHT

W. J. O'Neill

ATTORNEY

## UNITED STATES PATENT OFFICE

2,157,701

## PIEZOELECTRIC APPARATUS

Stuart C. Hight, South Orange, N. J., assignor  
to Bell Telephone Laboratories, Incorporated,  
New York, N. Y., a corporation of New York

Application May 19, 1936, Serial No. 80,513

13 Claims. (Cl. 171—327)

This invention relates to piezoelectric apparatus and particularly to piezoelectric crystals suitable for use as circuit elements in oscillation generator systems and in electric wave filter systems, for example.

One of the objects of this invention is to produce a piezoelectric crystal element that may have substantially zero or other desired predetermined temperature coefficient of oscillation frequency either positive or negative and that may be of a convenient size and shape and yet have a relatively low frequency vibration in the range from 30 to 1000 kilocycles per second, for example.

Another object of this invention is to produce a piezoelectric body that may have a frequency substantially independent of changes in temperature over a substantial range of temperatures to permit temperature regulating apparatus to be simplified or eliminated and to permit a constant vibration frequency to be maintained.

Another object of this invention is to obtain for a piezoelectric body a predetermined temperature coefficient of frequency that may have a positive, negative or zero value.

Another object of this invention is to increase the piezoelectric activity of a crystal oscillator.

It is well known that a quartz oscillator may produce an oscillation of fairly constant frequency and yet there may exist various factors affecting the constancy of oscillation frequency. Among them, the variation of the operating temperature of the crystal is an important factor. It is desirable therefore to obtain a crystal having its oscillation frequency independent of the temperature variation.

In accordance with this invention, the temperature coefficient of frequency of a piezoelectric crystal may be made to pass through zero or go to a positive value. The zero temperature coefficient of frequency may be obtained accurately enough for frequency standard purposes. This result may be obtained by a suitable selection of the orientation, shape, ratio of dimensions and mode of vibration of the crystal.

In a particular embodiment, the crystal may be in the shape of a rectangular parallelepiped having its longest or major axis dimension substantially perpendicular to an electric or X axis thereof and inclined with respect to the mechanical or Y axis at an angle between about +5 degrees and +20 degrees or preferably about +10 degrees. The dimensional ratios of width to length and of thickness to length may be adjusted to proper values and the crystal operated in a suitable mode of vibration to obtain the zero value of tempera-

ture coefficient of frequency. The mode of vibration may be of longitudinal type at the fundamental or at a harmonic frequency along the longest dimension of the crystal to obtain the zero temperature coefficient of frequency. The harmonic frequency may be the second, third, or fourth harmonic, for example. The second harmonic longitudinal vibration in the Y' direction of the crystal provides a very active piezoelectric oscillator. The harmonic vibration may be obtained by a suitable number of pairs of interconnected electrodes corresponding in number of pairs to the order of the selected harmonic.

For a clearer understanding of the nature of this invention and the additional features and objects thereof, reference is made to the following description taken in connection with the accompanying drawings, in which like reference characters represent like or similar parts and in which:

Fig. 1 is a side view of crystal apparatus embodying this invention;

Fig. 2 is a perspective view of the crystal apparatus illustrated in Fig. 1;

Fig. 3 is a top view of the crystal apparatus illustrated in Fig. 1 adapted to control the frequency of an oscillation generator connected in circuit therewith;

Figs. 4, 5 and 6 are respectively top, elevation and end views of a holder suitable for mounting the crystal illustrated in Figs. 1 to 3;

Figs. 7, 8 and 9 are views of another form of holder and electrodes suitable for mounting the crystal illustrated in Figs. 1 to 3;

Fig. 10 is a graph showing the values of temperature coefficient of frequency of particular quartz crystals having selected dimensional ratios;

Fig. 11 is a graph showing the values of frequency constant of particular crystals having selected dimensional ratios; and

Fig. 12 is a graph showing values of temperature coefficient of frequency and of frequency for particular crystals embodying this invention.

This specification will follow the standard terminology as applied to quartz which employs orthogonal X, Y and Z axes to designate the electric, the mechanical and the optic axes respectively of the piezoelectric crystal material and which employs X', Y' and Z' to designate the directions of axes or surfaces of a piezoelectric body angularly oriented with respect to the orthogonal X, Y and Z axes thereof. Where the orientation is obtained by rotation about an electric or X axis as particularly illustrated herein, the orientation

angle  $\theta$  designates the effective angular position of the crystal in degrees as measured from the mechanical or Y axis.

The dimensional ratio

$$5 \quad \frac{X}{Y'}$$

herein particularly illustrated, represents the dimensional ratio of thickness X in the direction of the X or electric axis of the crystal with respect to the length Y' or longest axis in the direction of the Y' axis; and the dimensional ratio

$$15 \quad \frac{Z'}{Y'}$$

15 represents the dimensional ratio of width Z' in the direction of the Z' axis with respect to the length in the direction of the Y' axis.

Quartz crystals may occur in two forms, namely, right-hand and left-hand. A crystal is 20 designated as right-hand if it rotates the plane of polarization of plane polarized light traveling along the optic or Z axis in a clockwise direction when facing in the direction of propagation of the light and is designated as left-hand if it rotates 25 the plane of polarization in the counter-clockwise direction. If a compressional stress be applied to the ends of the electric axis of a quartz crystal body and not removed, a charge will be developed 30 which is positive at the positive end of the electric axis and negative at the negative end of the electric axis for either right-hand or left-hand crystals. The magnitude and sign of the charge 35 may be measured with a vacuum tube electrometer, for example. In specifying the orientation of the right-hand crystal, the angle  $\theta$  which the new axis Z' makes with the optic axis Z as the crystal plate is rotated about the electric axis X is deemed positive when, with the positive end 40 of the X axis pointed toward the observer, the rotation is in a clockwise direction. A counter-clockwise rotation of such a crystal gives rise to a negative orientation angle. Conversely, the orientation angle of a left-hand crystal is positive when, with the positive end of the electric axis 45 X pointed toward the observer, the rotation is counter-clockwise and is negative when the rotation is clockwise. In one species of the invention as applied to quartz, the principal axis of the crystal is perpendicular to an X or electric axis 50 thereof and is oriented or inclined at a positive angle of approximately +10 degrees with respect to the mechanical axis thereof. In other species the principal axis may be inclined at an angle 55 between +5 and +20 degrees with respect to the mechanical or Y axis.

Referring to the drawings, Figs. 1 to 3 illustrate a right-hand piezoelectric quartz crystal 1 of substantially rectangular parallelepiped shape having its length dimension or longest axis Y' disposed substantially perpendicular to an X or electric axis thereof and inclined substantially  $\theta=+10$  degrees with respect to the mechanical or Y axis thereof. The width dimension Z' of the crystal 1 is disposed substantially perpendicular to the electric axis X and is axially inclined  $\theta=+10$  degrees with respect to the optic axis Z of the crystal 1 as illustrated in Fig. 1. In Fig. 1, the electric axis X is perpendicular to the plane of the drawing with the +X axis directed or projected into the plane of the paper. In Fig. 3, the electric axis X of the crystal 1 is parallel to the plane of the drawing and extends in the direction of the thickness dimension of the crystal 1 as indicated in Fig. 2. The crystal 1 is accordingly

a quartz bar having its principal axis oriented substantially +10 degrees with respect to the mechanical axis Y by rotation about the electric axis X and having the opposite electrode surfaces thereof disposed substantially perpendicular to the electric axis X thereof.

While the orientation angle  $\theta=$ substantially +10 degrees is a preferred orientation for the particular crystal illustrated in Figs. 1 to 3, it will be understood that a suitable orientation may be obtained between about  $\theta=+5$  and +20 degrees, for example.

Two pairs of opposite electrodes 10 to 13, one pair being the opposite electrodes 10 and 11 and the other pair being the opposite electrodes 12 and 13, may be interconnected by suitable conductive connectors as the connectors 15 and 16 illustrated in Fig. 3, for example, and utilized to apply an electric field to the crystal 1 in the direction of the electric axis X to excite the second harmonic 20 of the longitudinal mode of vibration substantially in the direction of the length axis Y' of the crystal 1.

The four electrodes 10 to 13 may be flat plates of stainless steel or other suitable conductive material disposed on or adjacent the two opposite surfaces of the crystal 1; or alternatively the electrodes 10 to 13 may be aluminum or other suitable metallic plating intimately adhering to and integral with the two opposite surfaces, as 30 shown, of the crystal 1.

The connector 15 interconnecting the electrodes 11 and 12 and the connector 16 interconnecting the electrodes 10 and 13 are illustrated in Fig. 3 as wire connectors but it will be understood that 35 they may be of any suitable construction such as, for example, metallic plating integral with the surfaces of the crystal 1.

Conductive connectors 18 and 19 connected respectively with the crystal electrodes 12 and 13 40 may be provided to connect the crystal 1 in circuit with a vacuum tube oscillation generator 20 as illustrated in Fig. 3, for example, to control the frequency of oscillations thereof. The particular oscillator 20 may include a vacuum tube 45 21 having a cathode 22, a grid electrode 23, and a plate electrode 24. The output circuit thereof may include a tuning coil 25 connected in parallel circuit relation with a variable condenser 26. A by-pass condenser 27 may connect the mid-point 50 of the tuning coil 25 with the cathode 22. A feed-back condenser 28 may feed back radio frequency oscillations to the grid electrode 23. Suitable batteries as illustrated may be provided to energize the cathode 22 and the plate electrode 24 in 55 a known manner. A grid leak resistance 29 and a milliammeter M may be connected between the grid 23 and the cathode 22. It will be understood that the crystal 1 may be utilized to control the frequency of oscillations of any suitable oscillator, the particular oscillator 20 being shown in Fig. 3 as an illustrative example only.

Similarly, the connectors 18 and 19 may connect the crystal 1 in circuit with an electric wave filter system to operate as a selective element 65 thereof.

Figs. 4, 5 and 6 illustrate respectively top, elevation and end views of a crystal holder or mounting which may be utilized for clamping rigidly at the nodes of motion and establishing 70 electrical connections with the second harmonic crystal 1 illustrated in Figs. 1 to 3. In this arrangement, two pairs of coaxial metallic clamping projections 30, 31 and 32, 33 disposed in contact with the four corresponding crystal elec- 75

trodes 10, 11, 12 and 13, respectively, and suitably supported from four posts 35 secured to an insulating base 36 by screws 37, for example, may rigidly nodally clamp the crystal 1 along the central longitudinal axis Y'Y' thereof at points or small areas located substantially one-quarter ( $\frac{1}{4}$ ) the length thereof from the small ends of the crystal 1 as illustrated in Figs. 1 to 6. The clamping projections 30 and 32 may slide freely in openings in the corresponding supporting posts 35 and be provided with suitable flanges 38 and coil springs 39 to resiliently clamp the crystal 1 between the clamping projections 30 to 33. The clamping projections 31 and 33 may have suitable screw threads thereon engaging the surfaces of openings in the corresponding supporting posts 35 to adjust the degree of clamping pressure exerted by the springs 39 on the crystal 1. Electrical connections between the metallic coated electrodes 11, 12 and 10, 14 respectively, may be indirectly established by conductive connectors 40 and 41 interconnecting the metallic clamping projections 31, 32 and 30, 33 respectively, or may be directly established as described and illustrated in connection with the conductors 15 and 16 in Fig. 3. The conductors 18 and 19 may connect the electrodes 12 and 13, respectively, with an oscillation generator such as the oscillation generator 20 illustrated in Fig. 3, or with any other desired system such as an electric wave-filter system, or other radio apparatus.

Figs. 7 and 8 are top views and Fig. 9 is a side view of another form of holder which may be utilized for mounting and establishing electrical connections with the crystal 1 shown in Figs. 1 to 3. In this arrangement, the crystal 1 may be supported within a rectangular opening in an insulating block 50 by means of the four flat electrodes 10 to 13, which may in this instance be pivotally attached to the block 50 by two pivot pins 51 and 52. Fig. 7 shows the electrodes 10 to 13 swung into open position to expose the crystal 1. Fig. 8 is a view similar to Fig. 7 but showing the electrodes 10 to 13 swung into operative relation with the crystal 1. The pin 51 may interconnect the crystal electrodes 11 and 12 and the pin 52 may interconnect the electrodes 10 and 13 to excite the second harmonic longitudinal vibration in the length direction Y' of the crystal 1 as illustrated in Fig. 3. Wedge-shaped projections 55 to 58 may be supported by the holder block 50 in any suitable manner and may make contact with small areas of the opposite surfaces of the crystal 1 on the nodal lines 59 and 60 thereof, as illustrated in Figs. 1 to 7, hold the crystal 1 in fixed position between the electrodes 10 to 13, which may be spaced in close relation to or in contact with opposite electrode surfaces of the crystal 1. The projections 55 to 58 may, if desired, be made resiliently adjustable with respect to the holder box 50 to adjust the clamping pressure exerted by the springs on the crystal 1 at the nodes 59 and 60 thereof. The nodal lines for the crystal 1 shown in Figs. 1 to 3 are substantially in the positions shown therein. The electrodes 10 to 13 may be swung about the pivots 51 and 52 to open position as illustrated in Fig. 7 to remove or insert the crystal 1.

By giving certain selected values to both the dimensional ratios of width to length

and of thickness to length

$$\frac{X}{Y'}$$

of the crystal 1, the longitudinal mode of vibration therein may be mechanically coupled to other modes, as flexures and transverse modes of vibration therein having positive temperature coefficients of frequency, to produce selected negative, positive or zero temperature coefficients of frequency for the crystal 1.

The dimensional ratios

$$\frac{X}{Y'} \text{ and } \frac{Z'}{Y'}$$

to obtain the desired predetermined temperature coefficient as the zero temperature coefficient of frequency will depend upon the orientation angle  $\Theta$  of the crystal 1 and the order of the harmonic operation thereof.

Where the crystal 1 has an orientation angle or angular position of  $\Theta$ =about +10 degrees rotated about an electric axis X and is excited by an electric field in the direction of the electric axis XX by the two pairs of electrodes 10 to 13 which drive the crystal 1 at the second harmonic or overtone of the longitudinal vibrations in the direction of the length or longest axis Y', all as illustrated in Figs. 1 to 3, the dimensional ratios

$$\frac{X}{Y'} \text{ and } \frac{Z'}{Y'}$$

of the crystal 1 to obtain zero or other predetermined temperature coefficient of frequency may be as illustrated by the curves given in Fig. 10.

For example, to obtain zero temperature coefficient of frequency in the second harmonic +10 degree crystal 1 illustrated in Figs. 1 to 3, the dimensional ratio

$$\frac{Z'}{Y'}$$

may be about .28 when the dimensional ratio

$$\frac{X}{Y'}$$

is about .300 as illustrated in curve A of Fig. 10; or the dimensional ratio

$$\frac{Z'}{Y'}$$

may be about .245 when the dimensional ratio

$$\frac{X}{Y'}$$

is about .223 as illustrated in curve B of Fig. 10. Curves C and D of Fig. 10 illustrate temperature coefficients of frequency that may be obtained for other values of dimensional ratios

$$\frac{X}{Y'} \text{ and } \frac{Z'}{Y'}$$

It will be noted that crystal apparatus constructed in accordance with this invention by suitable selection of the orientation, mode of vibration and dimensional ratios

$$\frac{X}{Y'} \text{ and } \frac{Z'}{Y'}$$

may have substantially precisely zero temperature coefficient of frequency or may have a selected positive or negative temperature coefficient of frequency as illustrated by curves A or B, for example, in Fig. 10.

Fig. 11 shows the values of the frequency constant in terms of kilocycles x centimeters of sec-

ond harmonic +10 degree crystals, as illustrated in Figs. 1 to 3, where one has a dimensional ratio

$$\frac{X}{Y'} = \text{about } .22$$

5 and another has a dimensional ratio

$$\frac{X}{Y'} = \text{about } .30$$

10 and both having various dimensional ratios

$$\frac{Z'}{Y'}$$

as indicated. The term, frequency constant, as used herein indicates the product of the frequency of the crystal bar  $I$  in kilocycles per second and the frequency determining length  $Y'$  thereof in centimeters. The curves A and B of Fig. 11 correspond to the curves A and B, respectively, of Fig. 10.

20 It will be noted from curves A and B, for example, in Figs. 10 and 11 that reducing the

$$\frac{Z'}{Y'}$$

25 dimensional ratio as, for example, by reducing the  $Z'$  dimension of the crystal  $I$  while holding the  $Y'$  dimension constant, lowers the frequency of the crystal  $I$  and at the same time makes the temperature coefficient of frequency thereof more positive. This property makes it possible to obtain zero temperature coefficient of frequency at any desired frequency, as will be illustrated in connection with Fig. 12 which shows in one graph the approximate relations between the  $Z'$  30 dimension, the  $Y'$  dimension, the frequency and the temperature coefficient of frequency of a second harmonic +10 degree quartz crystal  $I$  illustrated in Figs. 1 to 3, when  $X=0.22Y'$  corresponding to the curve B in Figs. 10 and 11.

35 Referring to Fig. 12, it will be noted that reducing the  $Z'$  dimensions of the crystal  $I$  decreases the frequency and, at the same time, makes the temperature coefficient of frequency more positive; while reducing the  $Y'$  dimension increases the frequency and, at the same time, makes the temperature coefficient of frequency more negative. The path shown by the broken line and arrows in Fig. 12 illustrates one way in which the crystal  $I$  shown in Figs. 1 to 3 may be 40 ground to obtain substantially precisely zero temperature coefficient of frequency at a desired frequency of 100 kilocycles per second, for example, assuming that the crystal  $I$  originally has properties as indicated at point A in Fig. 12. 45 At point A of Fig. 12, the length or  $Y'$  dimension of the crystal  $I$  is between 61 and 62 millimeters, the width or  $Z'$  dimension is between 16 and 17 millimeters, and the thickness or  $X'$  dimension is 0.22 $Y'$  and at point A the crystal  $I$  has a frequency of 95 kilocycles and a temperature coefficient of frequency between -2 and -3 50 parts per million per degree centigrade. Reducing the dimension  $Y'$  to between 58 and 59 millimeters, as indicated at B in Fig. 12, increases the frequency to the selected desired value of 100 kilocycles per second and at the same time makes the temperature coefficient of frequency more negative, bringing it to between -4 and -5 parts per million per degree centigrade. Reducing the dimension  $Z'$  to between 14 and 15 millimeters width for the crystal  $I$  as illustrated at point C in Fig. 12, lowers the frequency to about 99.4 kilocycles per second and, at the same time, makes the temperature coefficient of frequency more positive and brings it to the desired 75

zero value as indicated at point C in Fig. 12. The  $Y'$  dimension may then be further reduced until the desired frequency of 100 kilocycles is again obtained as indicated at point D in Fig. 12. Thus, by alternately reducing the  $Y'$  and  $Z'$  dimensions of the crystal  $I$  without exceeding, in the course of grinding, the desired frequency and temperature coefficient of frequency, and measuring the frequency and temperature coefficient of frequency at suitable intervals as the grinding proceeds, ultimately both the desired frequency and zero temperature coefficient of frequency as illustrated at point E of Fig. 12 may be obtained.

It will be noted that to obtain the 100 kilocycle zero temperature coefficient of frequency second harmonic crystal  $I$  illustrated at point E of Fig. 12, the length dimension  $Y'$  will be about 58.4 millimeters, the width dimension  $Z'$  will be about 0.25 $Y'$ , and the thickness dimension  $X$  will be about 0.22 $Y'$ , and that the frequency is given by the relation

$$\text{frequency} = \frac{5840}{Y'} \text{ kilocycles}$$

where  $Y'$  is the length of the crystal  $I$  in millimeters.

It will be noted that the orientation, as the +10 degree orientation illustrated in Fig. 1, determines the wave direction generally in the crystal  $I$ . The dimensional ratios of the width  $Z'$  and the thickness  $X$  with respect to the length  $Y'$  vary the wave direction somewhat and determine the amounts of coupling to other modes of vibration as flexures and transverse modes having positive temperature coefficients of frequency in order to produce the desired zero temperature coefficient of frequency for the crystal  $I$ .

The control of the temperature coefficient of frequency of the crystal  $I$  is such as to produce positive or negative coefficients at will and, therefore, to produce substantially precisely zero temperature coefficient of frequency and the dimensions of the crystal  $I$  are large enough to insure mechanical strength and contain enough volume of quartz to store sufficient vibrational energy to insure strong oscillations and good frequency control.

Operation on the second harmonic frequency as illustrated in Figs. 1 to 3 may provide certain advantages over operation on the fundamental or the higher order of harmonics as the third, fourth, or fifth harmonic, for example.

When operated on the second harmonic frequency as illustrated in Figs. 1 to 3, for example, the crystal  $I$  is very active as an oscillator and may be operated in an ordinary circuit having no additional feedback circuit. As a resonator, the second harmonic operation may offer a great increase in admittance, admittance being defined as the ratio of current to voltage at resonance or the reciprocal of the effective resistance of the crystal. The increase in the size of the crystal when operated at the second harmonic frequency may be advantageous at the higher frequencies. The two nodal lines, as the nodal lines 59 and 60, may be advantageous for clamping. The frequency constant, which is the frequency  $\times$  the length, of the second harmonic crystal  $I$  is twice that for the same crystal vibrated at the fundamental frequency and, therefore, twice the amount of quartz may be ground off the length dimension  $Y'$  to change the frequency by a given amount with resulting accuracy in grinding to a specified frequency.

The arrangement illustrated in Fig. 1 utilizes harmonic operation, orientation, and selected dimensional ratios to produce a crystal suitable for obtaining an extremely accurate frequency, 5 and having a convenient size, a high frequency constant, a high admittance, and two nodal lines or surfaces which may be utilized for rigidly clamping the crystal. Both the frequency and temperature coefficient of frequency may be 10 raised or lowered separately, insuring a substantially exact adjustment by simple procedure.

While particular dimensional ratios for a particular angular orientation of +10 degrees have been illustrated, it will be understood that the 15 optimum dimensional ratios of width to length and of thickness to length may be similarly obtained in order to secure zero temperature coefficient of frequency for other angular orientations with respect to the mechanical or Y axis. 20 While Figs. 1 to 3 illustrate a crystal I driven at the second harmonic of its length vibrations substantially in the direction of the Y' axis by means of two pairs of interconnected electrodes 10 to 13, it will be understood that the crystal 25 may be driven at another harmonic as the third or fourth harmonic of the length vibrations by means of a number of pairs of opposite electrodes similarly interconnected and corresponding in 30 number of pairs to the order of the harmonic desired as, for example, three pairs of opposite electrodes for the third harmonic frequency or four pairs for the fourth harmonic frequency or to drive the crystal at the fundamental length vibrations, one pair of opposite electrodes may 35 be utilized. When so driven at the fundamental or harmonic longitudinal mode of motion, the zero temperature coefficient of frequency may be obtained, as in the case of the second harmonic crystal illustrated in Figs. 1 to 3 by a suitable orientation and by selected dimensional 40 ratios

$$\frac{X}{Y'} \text{ and } \frac{Z'}{Y'}$$

45 to couple the longitudinal mode of vibration to other modes having positive temperature coefficients of frequency to produce zero temperature coefficient of frequency as described in connection with the example illustrated.

It will be understood that the crystal I driven 50 at an odd harmonic as, for example, the third, fifth or seventh harmonic may be centrally nodally clamped by a single pair of coaxial clamping projections, and may be utilized as a 55 selective element in an electric wave filter where constancy of frequency is desired independent of substantial temperature change.

Although this invention has been described and illustrated in relation to specific arrangements, it is to be understood that it is capable of 60 application in other organizations and is, therefore, not to be limited to the particular embodiments disclosed but only by the scope of the appended claims and the state of the prior art.

65 What is claimed is:

1. An elongated piezoelectric quartz crystal of substantially rectangular parallelepiped shape having opposite electrode surfaces and the longest axis thereof disposed substantially perpendicular to an X axis said longest axis being inclined substantially +10 degrees with respect to a Y axis thereof, and means comprising a plurality of pairs of opposite electrodes operatively disposed with respect to said crystal electrode 70 surfaces and interconnections between said elec-

trodes for operating said crystal at the second harmonic frequency of the mode of vibration thereof substantially in the direction of said longest axis, said crystal having selected dimensional ratios of width and of thickness with respect to said longest axis for mechanically coupling said harmonic mode of vibration to at least one other mode of vibration therein having positive temperature coefficient of frequency for obtaining zero temperature coefficient of frequency 10 for said crystal, said dimensional ratios being between 0.2 and 0.3.

2. An elongated piezoelectric quartz crystal of substantially rectangular parallelepiped shape having opposite electrode surfaces and the longest axis thereof disposed substantially perpendicular to an X axis said longest axis being inclined substantially +10 degrees with respect to a Y axis thereof, and means comprising a plurality of pairs of opposite electrodes operatively 15 disposed with respect to said crystal electrode surfaces and interconnections between said electrodes for operating said crystal at the second harmonic frequency of the mode of vibration thereof substantially in the direction of said longest axis, said crystal having selected dimensional ratios of width and of thickness with respect to said longest axis and being those determined substantially by the curves of Fig. 10 for mechanically coupling said harmonic mode of vibration to at least one other mode of vibration therein having positive temperature coefficient of frequency for obtaining a selected temperature coefficient of frequency for said crystal. 20

3. A piezoelectric quartz crystal element of substantially rectangular parallelepiped shape having its longest axis along a Y' axis substantially perpendicular to an X axis and inclined at such an acute angle of substantially +10 degrees with respect to a Y axis thereof, and having such selected dimensional ratios of both the width along a Z' axis and the thickness along said X axis thereof with respect to said longest axis as to mechanically couple an overtone frequency of the mode of vibration therein in the 45 direction of said longest axis with another mode of vibration therein for obtaining a selected temperature coefficient of frequency therefor, said dimensional ratios being those determined substantially by the curves of Fig. 10. 50

4. The method of adjusting to desired values the temperature coefficient of frequency and the frequency of a piezoelectric crystal having orthogonal X, Y' and Z' dimensions the Z' dimension making an angle of substantially +10 degrees with respect to the Z axis which includes alternately reducing the Y' dimension to such a value as to increase the frequency to the desired value without exceeding the desired value of frequency while making the 60 temperature coefficient of frequency more negative, and reducing the Z' dimension to such a value as to make the temperature coefficient of frequency more positive and of the desired value without exceeding the desired value of temperature coefficient of frequency, while decreasing the frequency. 65

5. An elongated piezoelectric quartz crystal bar of rectangular parallelepiped shape having orthogonal X, Y' and Z' dimensions of predetermined relative values determined substantially by the curves of Fig. 10, said Z' dimension making an angle of substantially +10 degrees with respect to the Z axis, said Y' dimension being reduced to such a value as to obtain the desired 70 75

- frequency for said bar and said Z' dimension being reduced to such a value as to obtain the desired temperature coefficient of frequency for said bar.
5. 6. A piezoelectric quartz crystal oscillating bar of substantially rectangular parallelepiped shape having orthogonal X, Y' and Z' dimensions, said Y' dimension being elongated, substantially perpendicular to an X axis and inclined substantially 10 degrees with respect to a Y axis, the ratio of said dimensions Z' to Y' being substantially .28 and the ratio of said dimensions X to Y' being substantially .3 to obtain substantially zero temperature coefficient of frequency when excited at the second harmonic of the longitudinal mode of vibration in the direction of said Y' dimension by an electric field having a component in the direction of said X axis.
7. A piezoelectric quartz crystal oscillating bar 20 of substantially rectangular parallelepiped shape having orthogonal X, Y' and Z' dimensions, said Y' dimension being elongated, substantially perpendicular to an X axis and inclined substantially 15 +10 degrees with respect to a Y axis, the ratio of said dimensions Z' to Y' being substantially .245 and the ratio of said dimensions X to Y' being substantially .223 to obtain substantially zero temperature coefficient of frequency when excited at the second harmonic of the longitudinal mode of vibration in the direction of said Y' dimension by an electric field having a component in the direction of said X axis.
8. A piezoelectric quartz crystal oscillating bar 30 of substantially rectangular parallelepiped shape having electrode faces substantially perpendicular to an X axis and having orthogonal X, Y' and Z' dimensions, said Y' dimension being elongated, substantially perpendicular to said X axis and inclined substantially +10 degrees with respect 35 to the nearest Y axis thereof, the ratio of said X dimension to said Y' dimension and the ratio of said Z' dimension to said Y' dimension being selected values between substantially .2 and .3 to give a predetermined characteristic when operated at the second harmonic of the longitudinal mode of vibration in the direction of said Y' dimension.
9. A piezoelectric oscillating quartz crystal element of substantially rectangular parallelepiped 40 shape having electrode faces substantially perpendicular to an X axis and having orthogonal X, Y' and Z' dimensions, said Y' dimension being elongated and inclined at an angle substantially +10 degrees with respect to the nearest Y axis thereof, said X, Y' and Z' dimensions having such relative proportions and being those determined substantially by the curves of Fig. 10 as to produce a desired temperature coefficient of frequency when said crystal is operating at the second harmonic of the longitudinal mode of vibration in the direction of said Y' dimension.
10. A piezoelectric oscillating quartz crystal having electrode faces substantially perpendicular to an X axis and having orthogonal X, Y' and Z' dimensions, said Y' dimension being elongated and inclined at an angle substantially +10 degrees with respect to the nearest Y axis thereof, said X, Y' and Z' dimensions having relative proportions determined substantially by the curves of Fig. 10.
11. A piezoelectric quartz crystal oscillator having its axis of greatest length substantially perpendicular to an electric axis and inclined at 15 an acute angle with respect to the optic axis thereof, characterized in this that said angle, and the dimensional ratios of width to said length and of thickness to said length of said crystal have such relative values as to produce a desired 20 temperature coefficient of frequency at a given harmonic of the longitudinal mode of vibration in the direction of said axis of said length said angle being substantially 80 degrees, said dimensional ratios of width to length and of thickness 25 to length being selected between substantially .2 and .3, and said vibration being the second harmonic of said longitudinal mode of vibration.
12. A piezoelectric crystal element of quartz adapted to vibrate at its second harmonic lengthwise mode of motion having substantially the shape of a rectangular parallelepiped, having its longest or length dimension along a Y' axis and having its two other dimensions along an X axis and a Z' axis, the orientation of the crystal element being such that the angle between the Z' axis and the Z axis is substantially +10 degrees and the dimensions in the X, Y' and Z' directions being those determined substantially by the curves of Fig. 10.
13. A piezoelectric crystal element of quartz adapted to vibrate at its second harmonic lengthwise mode of motion having substantially the shape of a rectangular parallelepiped, having its longest or length dimension along a Y' axis and 30 having its two other dimensions along an X axis and a Z' axis, the orientation of the crystal element being such that the angle between the Z' axis and the Z axis is substantially +10 degrees and the dimensions in the X, Y' and Z' directions 35 being those determined substantially by the curves of Fig. 10, said dimension in said Y' direction being reduced to such a length as to obtain a desired frequency for said element and said dimension in said Z' direction being reduced 40 to such a value as to obtain a desired temperature coefficient of frequency for said element.

STUART C. HIGHT.